

# United States Patent [19]

Kenney

[11] 3,854,952

[45] Dec. 17, 1974

[54] PHOTOSENSITIVE SILVER HALIDE  
COMPOSITION

[75] Inventor: John Thomas Kenney, Trenton, N.J.

[73] Assignee: Western Electric Company,  
Incorporated, New York, N.Y.

[22] Filed: Sept. 19, 1973

[21] Appl. No.: 398,719

[52] U.S. Cl..... 96/94 BF, 96/108, 96/109,  
252/213 R

[51] Int. Cl..... G03c 1/02

[58] Field of Search..... 96/94 BF, 95, 108, 109,  
96/107; 252/213 R

[56] References Cited  
UNITED STATES PATENTS

1,995,444 3/1935 Berry et al. .... 96/95

|           |         |                     |           |
|-----------|---------|---------------------|-----------|
| 2,839,405 | 6/1958  | Jones .....         | 96/107    |
| 2,950,972 | 8/1960  | Mueller et al. .... | 96/108    |
| 3,556,797 | 1/1971  | Pattijw et al. .... | 96/109    |
| 3,657,003 | 4/1972  | Kenney .....        | 117/120   |
| 3,767,590 | 10/1973 | Kenney .....        | 252/313 R |

Primary Examiner—Norman G. Torchin

Assistant Examiner—Alfonso T. Suro Pico

Attorney, Agent, or Firm—J. Rosenstock

[57] ABSTRACT

A photosensitive silver halide composition is disclosed. The composition comprises a silver halide deposited or sorbed on colloidal particles of a hydrous oxide of an element selected from the group consisting of Be, Mg, Ti, Zr, V, Cr, Mo, W, Mn, Fe, Co, Ni, Cu, Zn, Cd, Hg, Al, In, Si, Ge, Sn, Th and mixtures thereof.

12 Claims, No Drawings

## PHOTOSENSITIVE SILVER HALIDE COMPOSITION

### BACKGROUND OF THE INVENTION

#### 1. Field of the Invention

This invention relates to a photosensitive silver halide composition and a method of forming the composition and more particularly, to a composition comprising a silver halide deposited on suitable colloidal particles of a hydrous oxide.

#### 2. 1 Description of the Prior Art

Silver halide films for photography are made from silver halide dispersed in gelatin. The resultant gelatin films are dimensionally unstable due to both thermal expansion and water absorption. Where the silver halide is to be applied to a hydrophobic surface, the use of gelatin films thereof have not proved satisfactory due to the poor wettability attained. A gelatin-free silver halide film which is dimensionally stable, which is resistant to decomposition for relatively long periods of time and which is capable of wetting hydrophobic surfaces is desired and is an object of the subject invention.

### SUMMARY OF THE INVENTION

This invention relates to a photosensitive silver halide composition and a method of forming the composition and more particularly, to a composition comprising a silver halide deposited on suitable colloidal particles of a hydrous oxide.

The photosensitive silver halide composition is a wetting silver halide composition in that it is capable of (1) rendering a non-wettable surface wettable and (2) tenaciously adhering to the non-wettable or hydrophobic surface. The composition comprises a silver halide deposited or sorbed on colloidal particles of a hydrous oxide of at least one element selected from the group comprising Be, Mg, Ti, Zr, V, Cr, Mo, W, Mn, Fe, Co, Cu, Zn, Cd, Hg, Al, In, Si, Ge, Sn, Th. The method of forming such a composition includes combining a suitable silver salt, e.g.,  $\text{AgNO}_3$ , with a suitable stable aqueous wetting colloidal solution, formed by a controlled hydrolysis and nucleation reaction, comprising a halide ion and insoluble hydrous oxide particles of a selected element in its most stable oxidation state which does not oxidize in water in the presence of oxygen or reduce silver ions ( $\text{Be}^{+2}$ ,  $\text{Mg}^{+2}$ ,  $\text{Ti}^{+4}$ ,  $\text{Zr}^{+4}$ ,  $\text{V}^{+4}$ ,  $\text{V}^{+5}$ ,  $\text{Cr}^{+3}$ ,  $\text{Mo}^{+6}$ ,  $\text{W}^{+6}$ ,  $\text{Mn}^{+7}$ ,  $\text{Mn}^{+3}$ ,  $\text{Fe}^{+3}$ ,  $\text{Co}^{+2}$ ,  $\text{Cu}^{+2}$ ,  $\text{Ni}^{+2}$ ,  $\text{Zn}^{+2}$ ,  $\text{Cd}^{+2}$ ,  $\text{Hg}^{+2}$ ,  $\text{Al}^{+3}$ ,  $\text{In}^{+3}$ ,  $\text{In}^{+1}$ ,  $\text{Ti}^{+1}$ ,  $\text{Si}^{+4}$ ,  $\text{Ge}^{+4}$ ,  $\text{Sn}^{+4}$ ,  $\text{Bi}^{+3}$ , and  $\text{Th}^{+4}$ ). The particles have a size within the range of 10A to 10,000A and the hydrolysis reaction includes at least (1) dissolution of a salt of the selected element in an aqueous medium and (2) maintenance of the pH of the aqueous medium at a point where no flocculate results.

### DETAILED DESCRIPTION

The present invention is described primarily in terms of a wetting photosensitive silver halide composition and a method of forming such a composition. However, it will be understood that such description is exemplary only and is for purposes of exposition and not for purposes of limitation. It will be readily appreciated that the inventive concept described is equally applicable to wetting compositions comprising a photosensitive halide of an element other than silver, e.g., Hg.

A suitable silver salt is selected. A suitable silver salt is one which is water soluble and which is compatible with a suitable colloidal wetting solution, comprising a halide ion and an insoluble hydrous oxide of a selected element, with which the silver salt is destined to be combined. By compatible is meant that the silver salt is not reduced to metallic silver by the colloidal solution and the colloidal state of the solution is not destroyed by the addition of the silver salt thereto. The silver salt, e.g.,  $\text{AgNO}_3$ , is dissolved in water to form an aqueous solution typically in concentration of about 0.1-1.0 weight percent of  $\text{AgNO}_3$ . It is to be noted, however, that the concentration of the aqueous  $\text{AgNO}_3$  solution is not critical and the invention is not to be restricted thereby.

A suitable aqueous colloidal wetting solution comprising a halide ion and insoluble colloidal particles of a hydrous oxide is selected. A suitable colloidal wetting solution is a stable colloidal wetting solution formed by 20 a controlled hydrolysis and nucleation reaction in an aqueous medium wherein (1) colloidal particles of the colloidal solution have a size within the range of 10A to 10,000A, (2) colloidal particles of the colloidal solution comprise an insoluble hydrous oxide of one or 25 more elements selected from the group comprising Be, Mg, Ti, Zr, V, Cr, Mo, W, Mn, Fe, Co, Ni, Cu, Zn, Cd, Hg, Al, In, Tl, Si, Ge, Sn, Bi, and Th, (3) no species is present, atomic or ionic, including any species of the above enumerated element, which is capable of reducing 30 the silver salt, destined to be added thereto or combined therewith, to metallic silver, and (4) a halid ion is present. It is to be emphasized that the hydrous oxide is of an element in its most stable oxidation state which does not oxidize in water in the presence of oxygen or 35 reduce silver ions to metallic silver. Typical of such elemental oxidation states are  $\text{Be}^{+2}$ ,  $\text{Mg}^{+2}$ ,  $\text{Ti}^{+4}$ ,  $\text{Zr}^{+4}$ ,  $\text{V}^{+5}$ ,  $\text{V}^{+4}$ ,  $\text{Cr}^{+3}$ ,  $\text{Mo}^{+6}$ ,  $\text{W}^{+6}$ ,  $\text{Mn}^{+3}$ ,  $\text{Mn}^{+7}$ ,  $\text{Fe}^{+3}$ ,  $\text{Co}^{+2}$ ,  $\text{Ni}^{+2}$ ,  $\text{Cu}^{+2}$ ,  $\text{Zn}^{+2}$ ,  $\text{Cd}^{+2}$ ,  $\text{Hg}^{+2}$ ,  $\text{Al}^{+3}$ ,  $\text{In}^{+3}$ ,  $\text{In}^{+1}$ ,  $\text{Si}^{+4}$ ,  $\text{Ge}^{+4}$ ,  $\text{Sn}^{+4}$ ,  $\text{Bi}^{+3}$ , and  $\text{Th}^{+4}$ .

40 The term "hydrous oxide" is defined for purposes of the present invention as an insoluble oxide, an insoluble hydroxide, an insoluble oxide-hydroxide, or an insoluble mixture of an oxide and a hydroxide.

45 Moreover, the term "hydrous oxide" as used herein is intended to include all permutations and combinations of one or more of the following types of oxides and/or hydroxides:

50 1. True Hydrous Oxides—Those oxides which include an indefinite amount of  $\text{H}_2\text{O}$  in other than stoichiometric fashion. That is, a salt of a selected element + hydrous  $\text{H}_2\text{O}$ .

55 2. True Hydroxides — Those compounds of a salt which contain actual OH-groups. That is, a salt of a selected element + only sufficient stoichiometric  $\text{H}_2\text{O}$  to form a hydroxide.

60 3. Hydrous Hydroxides — True hydroxides which also contain hydrous  $\text{H}_2\text{O}$  in indefinite amounts. That is, a salt of a selected element + stoichiometric  $\text{H}_2\text{O}$  necessary to form a hydroxide + hydrous  $\text{H}_2\text{O}$ .

65 4. Hydrous hydrates — A salt of a selected element + some of the stoichiometric  $\text{H}_2\text{O}$  necessary to form a hydroxide + hydrous  $\text{H}_2\text{O}$ .

A more detailed explanation of the term "hydrous oxide" is contained in both *Inorganic Colloid Chemistry* by H. B. Weiser, Vol. 11, "The Hydrous Oxides and Hydroxides," Chapter I, John Wiley and Sons, Inc., New York (1935); and *Inorganic Chemistry, An Advanced*

*Textbook by T. Moeller, John Wiley and Sons, Inc., New York (1952).*

It should be noted that the term "hydrous H<sub>2</sub>O" refers to water carried by the compound in other than stoichiometric fashion. Specifically, such water is probably not carried in chemical fashion but is rather surface sorbed, occluded or held as a part of the unit crystal.

The hydrolysis reaction includes dissolving a salt of the selected element in the aqueous medium and maintaining the pH of the aqueous medium at a point where no flocculate results.

Suitable colloidal solutions include some of the colloidal wetting solutions revealed in U.S. Pat. No. 3,657,003, filed Feb. 2, 1970, assigned to the assignee hereof and incorporated by reference herein. More specifically, the following solutions disclosed in U.S. Pat. No. 3,657,003 are some suitable colloidal wetting solutions for purposes of this invention:

1. The colorless (light, milky white) colloidal wetting solution of Example I-A which is obtained by (a) dissolving ½ weight percent of beryllium chloride [BeCl<sub>2</sub>] in 100 ml. of deionized water and (b) raising the initial pH of 3.0 to a value of 5.6-5.8 by adding dilute NH<sub>4</sub>OH (H<sub>2</sub>O dilution of 1/20) thereto;

2. The colorless (light, milky white) wetting solution of Example I-B which is obtained by (a) dissolving 1 weight percent of beryllium chloride [BeCl<sub>2</sub>] in 100 ml. of deionized water and (b) raising the initial pH with NaOH to about 5;

3. The colorless (light, milky white) wetting solution of Example I-C which is obtained by (a) adding ¼ to ½ weight percent of beryllium chloride [BeCl<sub>2</sub>] to 100 ml. of deionized water and (b) heating the resultant solution for about 1 hour at 70°C;

4. The colorless (light, milky white) wetting solution of Example II-A which is obtained by (a) dissolving 1 weight percent of magnesium chloride [MgCl<sub>2</sub> or MgCl<sub>2</sub>.6H<sub>2</sub>O] in 100 ml. of deionized water and (b) raising the initial pH with univalent alkali to about 8;

5. The yellow wetting solution of Example III-C which is obtained by (a) adding particulated titanium metal (Ti<sup>0</sup>) to a hot or boiling (about 80°C) concentrated univalent acid, such as HCl, until 0.2-3 weight percent of the titanium is dissolved, (b) allowing the solution to cool to room temperature, (c) adding sufficient H<sub>2</sub>O<sub>2</sub> to quantitatively render all the dissolved titanium (Ti<sup>+3</sup>) to Ti<sup>+4</sup> and (d) raising the pH with a univalent alkali, such as NaOH, to the range of about 1.2-2.0;

6. The blue wetting solution of Example III-D which is obtained by (a) adding particulated anhydrous titanium trichloride [TiCl<sub>3</sub>] to a concentrated univalent acid diluted with deionized water 1 weight percent of the titanium trichloride is dissolved and (b) raising the initial pH to about 10 with a univalent alkali, such as NaOH, to form TiO<sub>2</sub>;

7. The murky, pale yellow wetting solution of example III-E which is obtained by (a) adding one gram of fused titanium metal [Ti<sup>0</sup>] to 70 ml. of concentrated HCl, (b) boiling the resultant solution until it assumes a pale blue color, (c) heating the solution without boiling until most or all of the titanium metal has been dissolved and reacted to obtain a blue-purple solution having a very low pH, (d) raising the pH to about 0.5 with 1N-NaOH to obtain a pale lavender solution, (e)

adding dilute 50% H<sub>2</sub>O<sub>2</sub> to the solution to render it colorless (adding 1-2 drops in excess), and (f) raising the pH to about 1.0-1.2 with 1N-NaOH;

8. The wetting solution of Example III-F which is obtained by adding 0.1-5 weight percent of solid particulated (about 100A) titanium dioxide [TiO<sub>2</sub>] to water;

9. The wetting solution of Example III-G which is obtained by (a) adding 0.5-5 weight percent of titanium tetrachloride [TiCl<sub>4</sub>] to concentrated HCl and (b) slowly raising the initial pH of the resultant solution by the addition thereto of H<sub>2</sub>O or a dilute base such as NaOH or NH<sub>4</sub>OH to a pH of 0.5-5;

10. The colorless (light, milky white) wetting solution of Example IV which is obtained by (a) dissolving 1 weight percent zirconyl chloride [ZrOCl<sub>2</sub>.H<sub>2</sub>O] in 100 ml. of deionized water, (b) when the initial pH of the resultant solution is less than 1, heating the solution or adding thereto NaOH until the pH is about 1.4-2, or alternatively, if the pH is greater than 1 the pH is lowered to 1 or less with a univalent acid, such as HCl, and (c) either heating or adding NaOH until the pH is about 1.4-2;

11. The red-brown wetting solution of Example V-A which is obtained by (a) dissolving 1 weight percent of vanadium oxychloride [VOCl] in 100 ml. of hot or boiling concentrated univalent acid such as HNO<sub>3</sub>, (b) raising the pH of the resultant solution to about 1.5-2 with a univalent alkali solution and (c) heating the solution and adding a small amount of H<sub>2</sub>O<sub>2</sub> thereto;

12. The red-brown colloidal wetting solution of Example V-B which is obtained by (a) dissolving 1 weight percent of sodium vanadate [NaVO<sub>3</sub>], potassium vanadate [KVO<sub>3</sub>] or ammonium meta-vanadate [NH<sub>4</sub>VO<sub>3</sub>] in 100 ml. of deionized water and (b) lowering the initial alkaline pH of the solution to a value of about 5-6 with HCl;

13. The brown-red colloidal wetting solution of Example V-C which is obtained by (a) adding 1/2 weight percent of vanadium tetrachloride [VCl<sub>4</sub>] to concentrated HCl and (b) slowly raising the pH to about 1, e.g., by diluting with H<sub>2</sub>O;

14. The wetting solution of Example VI which is obtained by (a) dissolving 1/2 weight percent of green chromic chloride [CrCl<sub>3</sub>.6H<sub>2</sub>O], but probably more properly [Cr(H<sub>2</sub>O)<sub>4</sub>Cl<sub>2</sub>]Cl.2H<sub>2</sub>O or [Cr(H<sub>2</sub>O)<sub>5</sub>Cl].6-H<sub>2</sub>O] in 100 ml. of deionized water and (b) raising the initial pH of the resultant solution to about 5 with a univalent alkali;

15. The slightly yellow wetting solution of Example VII which is obtained by (a) dissolving 1 weight percent of sodium molybdate [Na<sub>2</sub>MoO<sub>4</sub>.2H<sub>2</sub>O or Na<sub>4</sub>(-6Mo<sub>7</sub>O<sub>24</sub>).4H<sub>2</sub>O] in 100 ml. of deionized water and (b) lowering the initial pH with a HCl to just below 7;

16. The faint yellow wetting solution of Example VIII which is obtained by (a) dissolving 1-5 weight percent of sodium tungstate dihydrate [Na<sub>2</sub>WO<sub>4</sub>.2H<sub>2</sub>O] in 100 ml. of deionized water and (b) lowering the pH with a HCl to below 1;

17. The muddy brown wetting solution of Example IX-B which is obtained by (a) dissolving 1 weight percent of manganese trichloride [MnCl<sub>3</sub>] in sufficient HCl to produce a solution having a pH of about 0.5-2, (b) adding excess H<sub>2</sub>O<sub>2</sub> thereto and (c) heating the resultant solution and raising the pH to 0.6-8 with NaOH. This same procedure may be followed with manganese dichloride;

18. The tan wetting solution of Example X-A which is obtained by dissolving 1 weight percent of ferric chloride  $[FeCl_3 \cdot 6H_2O]$  in 100 ml. of deionized water, the dissolution being added by gradually heating to about 50–80°C and stirring to obtain a wetting solution at a pH of 1.7–1.9;

19. The wetting solution of Example X-B which is obtained by (a) dissolving 0.5–5 weight percent of ferric chloride  $[FeCl_3 \cdot 6H_2O]$  in 100 ml. of deionized water, (b) adjusting the final pH of the resultant solution to about 1.5–2.0 with either HCl (at low ferric chloride concentrations) or NaOH (at high ferric chloride concentrations) and (c) heating the solution to 70°C within 20 minutes;

20. The wetting solution of Example X-C which is obtained by (a) dispersing 1.5 weight percent of ferric chloride  $[FeCl_3 \cdot 6H_2O]$  in 100 ml. of deionized water to a final pH of about 1.7–1.9 and (b) allowing the resultant solution to stand in ambient for 1–2 weeks;

21. The wetting solution of Example X-D which is obtained in the same manner as Examples X-B and X-C, described above [(19) and (20)], except that ferric bromide  $[FeBr_3 \text{ or } FeBr_3 \cdot 6H_2O]$  is employed;

22. The wetting solution of Example X-E which is obtained by dissolving 0.5–5 weight percent of ferric chloride  $[FeCl_3 \cdot 6H_2O]$  in 100 ml. of deionized water which was first heated to 70°C;

23. The wetting solution of Example X-F which is obtained by (a) adding 1 weight percent of ferric oxide  $[Fe_2O_3]$  which was particulated and powdered to a particulate size of about 150A in 100 ml. of deionized water, (b) ultrasonically agitating the mixture to aid in the dissolution of the ferric oxide and (c) lowering the pH of the resultant solution from 3–3.5 to 1.0 with HCl;

24. The wetting solution of Example X-G which is obtained by (a) adding 1 weight percent of ferric oxide  $[Fe_3O_4]$  which was particulated and powdered to a particulate size of about 150A in 100 ml. of deionized water, (b) ultrasonically agitating the mixture to aid in the dissolution of the ferric oxide  $[Fe_3O_4]$  and (c) lowering the pH of the resultant solution from 3–3.5 to 1.0 with HCl;

25. The wetting solution of Example X-H which is obtained by (a) heating 100 ml. of deionized water to 80°C and (b) adding 1–2 weight percent of ferric chloride  $[FeCl_3 \cdot 6H_2O]$  to the deionized water with stirring until dissolution occurs;

26. The blue wetting solution of Example XI-A which is obtained by (a) dissolving 1 weight percent of cobaltous chloride  $[CoCl_2 \cdot 6H_2O]$  in 100 ml. of deionized water and (b) raising the pH from 4.9–5.1 to about 7.0–7.2 with 1N-NaOH;

27. The wetting solution of Example XI-B which is obtained by (a) adding 1 weight percent of cobaltous chloride  $[CoCl_2 \cdot 6H_2O]$  to 100 ml. of deionized water, (b) adding sufficient NaOH to the resultant solution to effect the onset of a Tyndal cone and (c) heating the solution to about 60–70°C for 2 days while adjusting the pH, as necessary, with NaOH to about 4;

28. The wetting solution of Example XI-C which is obtained by (a) adding 1 weight percent of cobaltous chloride  $[CoCl_2 \cdot 6H_2O]$  to 100 ml. of deionized water, (b) heating the resultant solution to about 60–70°C with constant stirring, (c) raising the pH to about 2 with NaOH, (d) heating the solution again and raising the pH again to about 2 and (e) continuing the above procedure until the onset of a Tyndal cone or for about

6 hours (the resultant wetting solution has a life of about one hour);

29. The green wetting solution of Example XII-A which is obtained by (a) dissolving one weight percent of nickel chloride  $[NiCl_2 \cdot 6H_2O]$  in 100 ml. of deionized water, (b) adding sufficient NaOH to effect the onset of a Tyndal cone and (c) heating the solution at about 60–70°C for 2 days keeping the pH adjusted to about 4 with NaOH;

30. The pale green wetting solution of Example XII-B which is obtained by (a) dissolving 1 weight percent of nickel chloride  $[NiCl_2 \cdot 6H_2O]$  in deionized water and (b) raising the pH of the resultant solution to about 6–6.5 with NaOH;

31. The blue wetting solution of Example XV which is obtained by (a) dissolving 1 weight percent of cupric chloride  $[CuCl_2]$  in 100 ml. of deionized water and (b) heating the resultant solution to about 70°C while continually adjusting the pH to about 6 with NaOH;

32. The wetting solution of Example XVIII which is obtained by (a) dissolving 1 weight percent of zinc chloride  $[ZnCl_2]$  in 100 ml. of deionized water, (b) adding a sufficient amount of a univalent alkali, such as NaOH, to effect a slight precipitate at a pH of about 4, (c) heating the resultant solution at 60–80°C until the precipitate dissolves, (d) adding dilute univalent alkali, such as NaOH, until the onset of a Tyndal cone, and finally, (e) the heating and acid addition steps are repeated until a colloidal solution results;

33. The wetting solution of Example XIX which is obtained by (a) dissolving 1 weight percent of cadmium chloride  $[CdCl_2 \cdot \frac{1}{2}H_2O]$  in 100 ml. of deionized water and (b) slowly raising the pH of the resultant solution (over several hours time) to about 8–9 with a very dilute univalent alkali, such as NaOH, during which time the solution is slightly (about 30–40°C) heated;

34. The yellow wetting solution of Example XX which is obtained by (a) dissolving 1 weight percent of mercuric chloride (corrosive sublimate)  $[HgCl_2]$  in 100 ml. of deionized water and (b) slowly adding a dilute univalent alkali, such as NaOH, to raise the pH to about 5;

35. The wetting solution of Example XXI-A which is obtained by (a) adding 1 weight percent of finely powdered aluminum chloride  $[AlCl_3]$  to 100 ml. of deionized water, (b) raising the pH to about 5.2 with a univalent alkali such as NaOH and (c) heating the resultant solution for about 2 hours at about 60–80°C;

36. The wetting solution of Example XXI-B which is obtained by (a) heating 100 ml. of deionized water to about 60°C, (b) adding 1 weight percent of aluminum chloride  $[AlCl_3 \cdot H_2O]$  thereto and (c) while the solution is still hot raising the pH from 2.5 to about 5.0–5.2 with a univalent alkali, such as 1N-NaOH;

37. The wetting solution of Example XXII-A which is obtained by (a) dissolving 1 weight percent of indium trichloride  $[InCl_3]$  in 100 ml. of deionized water and (b) raising the pH of the resultant solution to about 3 with NaOH;

38. The whitish wetting solution of Example XXII-B which is obtained by (a) dissolving  $\frac{1}{2}$  weight percent of indium monochloride  $[InCl]$  in 100 ml. of deionized water and (b) raising the pH to about 3.9 with dilute (factor of 20 with  $H_2O$ )  $NH_4OH$ ;

39. The yellow wetting solution of Example XXIII which is obtained by (a) adding 0.1 weight percent of

thallium monochloride [TlCl] to 100 ml. of deionized water, (b) raising the pH of the resultant solution to about 7.5-8 with NaOH and (c) adding a few ml. of dilute potassium ferricyanide [K<sub>3</sub>Fe(CN)<sub>6</sub>] to the solution with stirring;

40. The wetting solution of Example XXIV which is obtained by (a) adding 0.1-5 weight percent of silicon tetrachloride or tetrachlorosilane [SiCl<sub>4</sub>] to concentrated HCl and (b) stirring the resultant solution;

41. The colloidal wetting solution of Example XXV which is obtained by (a) adding 1-2 weight percent of germanium tetrachloride [GeCl<sub>4</sub>] to concentrated HCl and (b) diluting the resultant solution with H<sub>2</sub>O to raise the pH to about 0.5;

42. The wetting solution of Example XXVI-A which is obtained by (a) dissolving 1-3 weight percent of stannic chloride [SnCl<sub>4</sub>.5H<sub>2</sub>O] in 100 ml. of deionized water and (b) permitting the resultant solution to stand at room temperature for 1-3 days or at an elevated temperature (about 60°C) for about 1 hour until a flocculate forms. The supernatant portion is a wetting solution;

43. The wetting solution of Example XXVI-B which is obtained by (a) dissolving ½ weight percent of stannic chloride [SnCl<sub>4</sub>.5H<sub>2</sub>O] in 100 ml. of deionized water and (b) permitting the solution of stand for about 1 month until the pH thereof is about 0.8-1.8 and a flocculate forms at the bottom thereof. The supernatant portion of this solution is the wetting solution;

44. The colorless wetting solution of Example XXVI-C which is obtained by adding sufficient HCl to the bottom layer (containing the flocculate) of the solution of Example XXVI-B, described above, to lower the pH to about 0.8-1.8;

45. The colorless wetting solution of Example XXVI-D which is obtained by heating to 30-90°C for about 30 minutes the bottom layer (containing the flocculate) of the solution of Example XXVI-B, described above;

46. The wetting solution of Example XXVI-E which is obtained by (a) dissolving 1 weight percent of sodium hydroxo stannate [Na<sub>2</sub>SnO<sub>3</sub>.3H<sub>2</sub>O or Na<sub>2</sub>Sn(OH)<sub>6</sub>] in 100 ml. of deionized water and (b) lowering the pH of the resultant solution to about 7.5-8.5 by the slow addition of HCl;

47. The colorless (milky white) wetting solution of Example XXVIII which is obtained by (a) dissolving 1 weight percent of bismuth trichloride [BiCl<sub>3</sub>] in 100 ml. of dilute (pH about 0.2) HCl and (b) raising the pH of the resultant solution to about 3-4 with NaOH; and

48. The colorless wetting solution of Example XXXI which is obtained by (a) dissolving 1 weight percent of thorium chloride [ThCl<sub>4</sub>] in 100 ml. of deionized water and (b) slowly adding a univalent alkali, such as NaOH, to raise the pH of the resultant solution to about 4.

The pH of the aqueous AgNO<sub>3</sub> solution is adjusted, when necessary, by means of a suitable acid, e.g., HNO<sub>3</sub>, or base, e.g., NH<sub>4</sub>OH, to match the pH of the suitable colloidal solution with which it is destined to be combined. Following the pH adjustment, if required, the aqueous AgNO<sub>3</sub> solution is added to a selected suitable colloidal solution comprising a halide ion and insoluble colloidal hydrous oxide particles of a particular element. Upon the addition of the aqueous AgNO<sub>3</sub> solution, a reaction occurs between the Ag<sup>+</sup> ions and the halide ion, e.g., Cl<sup>-</sup>, Br<sup>-</sup>, I<sup>-</sup>, contained in the colloidal

solution whereby a silver halide, e.g., AgCl, AgBr, AgI, forms and is precipitated or deposited or sorbed on the individual colloidal hydrous oxide particles.

It is to be noted and stressed at this point that both the silver halide formed and the solution containing the silver halide are wetting, i.e., they both are capable of rendering a hydrophobic surface hydrophilic and also the silver halide composition formed is capable of adhering very well to the hydrophobic surface. In this regard, a film of the silver halide deposited on a hydrophobic surface, e.g., polytetrafluoroethylene, cannot be removed by the application of a cellophane adhesive tape peel test thereto. It is also to be noted and stressed at this point that usually upon the addition of an electrolyte to a colloidal solution flocculation of the colloid occurs destroying the colloidal solution and the properties associated therewith, e.g., wetting ability. Surprisingly, such has been found not to occur with the addition of the silver salt, e.g., AgNO<sub>3</sub>, to the above-described colloidal wetting solutions. The resultant solution retains both its colloidal state and its wetting ability (along with the formed silver halide).

Where the resultant silver halide composition is intended for photographic applications, a suitable support base, e.g., a cellulose support, a paper support, etc., is selected. Suitable support bases and the properties thereof depend upon the purpose of the photographic application. Such support bases are well known in the art to those skilled therein and will not be elaborated herein. The selected support base (hydrophilic or hydrophobic) is immersed in the resultant colloidal solution, comprising colloidal hydrous oxide particles having a silver halide deposit thereon, for a period of time sufficient to uniformly wet the surfaces thereof with the solution and deposit a uniform film of silver halide coated colloidal particles thereon. For most support bases an immersion of about one minute at 25°C is sufficient. In the case of a Teflon (polytetrafluoroethylene) support base, which is very hydrophobic and upon which a silver halide gelatin film cannot adequately adhere, an immersion of about 10 minutes is required.

It is to be noted that the amount of deposited film can be controlled by the length of time the surface or support base is immersed in the resultant wetting silver halide colloidal solution. The deposit can also be built up by removing the support base from the colloidal solution, rinsing, drying, heating at 60° to 120°C for 1-5 minutes and then repeating the sequence of steps starting with the immersion.

The support base is removed from the wetting silver halide containing colloidal solution, is rinsed in flowing deionized water and is then air dried. A surface coated with a wetting silver halide film is then selectively exposed to a source of suitable photographic light radiation to obtain a latent image comprising silver metal [Ag<sup>0</sup>] nuclei on those areas of the surface exposed. It is to be noted that the silver halide film coated surface is exposed to the light radiation for a period of time sufficient to form the latent image. Such a period of time is readily ascertained experimentally by one skilled in the art for a particular light source. It is to be noted, however, that the time of exposure is interdependent upon the intensity of the light source, i.e., upon the amount of energy transmitted by the source to the surface. This interdependency is well known in the art or is easily ascertained by one skilled therein. A typical

exposure may range from 1 to 10 millijoules/cm<sup>2</sup> at a wavelength ranging from 2000 to 3600A. It is to be pointed out that the wavelength dependence can be altered employing standard techniques well known in the art, e.g., by the use of various dyes.

The latent image is then developed using conventional silver halide photographic developers, including development of the silver halide by exposure to suitable radiation, which are well known to those skilled in the art and which will not be elaborated herein. Alternatively, the latent image can be physically developed by immersion in an electroless metal plating solution wherein the silver nuclei catalyze the reduction of electroless metal ions of electroless metal to obtain an electroless metal pattern corresponding to the latent image.

#### EXAMPLE I

A. A 1.0 weight percent aqueous AgNO<sub>3</sub> solution was prepared. The pH of the solution was adjusted with HNO<sub>3</sub> to a value of about 5. The resultant AgNO<sub>3</sub> solution was then added, in a concentration of 0.05 weight percent of the total solution, to a stable colloidal solution comprising (1) colloidal particles of a hydrous oxide of beryllium and (2) chloride ions, to form silver chloride which was deposited on or covered each of the individual colloidal beryllium hydrous oxide particles. The colloidal solution was prepared in the following manner. One weight percent of beryllium chloride [BeCl<sub>2</sub>] was added to and dissolved in 100 ml. of deionized water. The initial pH was raised with NaOH until it was about 5 whereat a Tyndal cone was observed.

A hydrophobic polyethylene terephthalate film, commercially obtained, was immersed in the resultant wetting silver chloride deposited colloidal solution for about 2 seconds at 25°C. The film was removed and rinsed in flowing deionized water for one minute whereafter it was air dried. This procedure was then repeated but with a hydrophobic polyimide film, commercially obtained. This procedure was repeated again but with a hydrophobic polytetrafluoroethylene film which was immersed in the resultant solution for 20 minutes.

A surface of each of the dried films (polyethylene terephthalate, polyimide and polytetrafluoroethylene), having a photosensitive layer comprising silver chloride deposited or coated colloidal beryllium hydrous oxide particles, was then selectively exposed to a source of ultraviolet radiation (1-10 millijoules/cm<sup>2</sup> intensity,  $\lambda = 2537\text{A}$ ). The light-exposed surface was then immersed in an electroless copper plating solution, commercially obtained, to obtain a 0.01 mil thick electroless copper deposit on the areas of each surface exposed to the light.

B. The procedure of Example I-A was repeated except that 0.5 weight percent (of the total weight of the resultant mixture) of AgNO<sub>3</sub> was added to the colloid solution.

A physical development comprising a 0.01 mil thick electroless copper pattern on each of the three respective film surfaces was obtained.

C. The procedure of Example I-A was repeated except that the beryllium hydrous oxide colloid particle containing solution was prepared in the following manner. One weight percent of beryllium chloride [BeCl<sub>2</sub>] was dissolved in 100 ml. of deionized water. The initial pH of the solution was raised with NaOH until it was

about 5 whereat a Tyndal cone was observed. A colorless (e.g., light, milky white) wetting solution was obtained. The pH of the aqueous AgNO<sub>3</sub> solution was adjusted to about 5 and was combined with the colloidal solution in a concentration of 0.05 weight percent AgNO<sub>3</sub>.

A physical development comprising a 0.01 mil thick electroless copper pattern on each of the three respective film surfaces was obtained.

10 D. The procedure of Example I-A was repeated except that the beryllium hydrous oxide colloid particle containing solution was prepared in the following manner. About 1/4 weight percent of beryllium chloride [BeCl<sub>2</sub>] was added to deionized water. The resultant solution was heated for about 1 hour at 70°C resulting in a colorless (light, milky white) colloid wetting solution. The aqueous AgNO<sub>3</sub> solution was adjusted to a pH of 5.0 prior to the addition thereof to the colloidal solution.

15 A physical development comprising a 0.01 mil thick electroless copper pattern on each of the three respective film surfaces was obtained.

#### EXAMPLE II

20 E. The procedure of Example I-A was repeated except that a colloid solution comprising colloidal hydrous oxide particles of magnesium was employed. The colloidal solution was prepared in the following manner. One weight percent of magnesium chloride [MgCl<sub>2</sub> or MgCl<sub>2</sub>.2H<sub>2</sub>O] was dissolved in 100 ml. of deionized water. The initial pH of the solution was then raised with a univalent alkali, i.e., NaOH to about 8. A colorless (light, milky white) wetting solution was produced. The aqueous AgNO<sub>3</sub> solution was added to the colloidal solution.

25 A physical development comprising a 0.01 mil thick electroless copper pattern on each of the three respective film surfaces was obtained.

40

F. The procedure of Example I-A was repeated except that a 1 weight percent aqueous AgNO<sub>3</sub> solution was prepared and added to a colloidal solution comprising colloidal hydrous oxide particles of chromium. The AgNO<sub>3</sub> was present in the resultant solution in a concentration of 0.5 weight percent. The colloidal solution was prepared in the following manner. One-half weight percent of a green chromic chloride [CrCl<sub>3</sub>.6H<sub>2</sub>O] was dissolved in 100 ml. of deionized water. The initial pH was raised to about 5 with NaOH to obtain a green wetting solution. Prior to combining the aqueous solutions, the pH of the AgNO<sub>3</sub> solution was adjusted to about 5 with HNO<sub>3</sub>.

45 A physical development evidenced by a 0.01 mil thick electroless copper pattern on each of the three respective film surfaces was obtained.

50 G. The procedure of Example III-A was repeated except that the AgNO<sub>3</sub> added to the colloidal solution was present in an amount of 0.01 weight percent. The results obtained were the same as in Example II-A above.

#### EXAMPLE IV

55 H. The procedure of Example I-A was repeated except that a 0.1 weight percent aqueous AgNO<sub>3</sub> solution was prepared. The aqueous AgNO<sub>3</sub> solution was combined with a stable aqueous colloidal solution comprising col-

loidal hydrous oxide particles of cobalt, The  $\text{AgNO}_3$  being present in a concentration of 0.01 weight percent. The colloidal solution was prepared in the following manner. One weight percent of cobaltous chloride [ $\text{CoCl}_2 \cdot 6\text{H}_2\text{O}$ ] was added to 100 ml. of deionized water to form a rose colored solution having a pH of about 4.9-5.1. The pH was then raised with 10%  $\text{NH}_4\text{OH}$  to about 7.5-7.8 to obtain a blue wetting solution.

A physical development evidenced by a 0.01 mil thick electroless copper pattern on each of the three respective film surfaces was obtained.

#### EXAMPLE V

The procedure of Example I-A was repeated except that the 0.1 weight percent aqueous  $\text{AgNO}_3$  solution was combined with a stable colloidal solution comprising colloidal hydrous oxide particles of copper, the  $\text{AgNO}_3$  being present therein in a concentration of 0.05 weight percent. The colloidal solution was prepared in the following manner. One weight percent of cupric chloride [ $\text{CuCl}_2$ ] was dissolved in 100 ml. of deionized water. The pH of the solution was raised by the slow addition of a 10% solution of  $\text{NH}_4\text{OH}$  to a pH of 7.2-7.5. This was a wetting solution.

A physical development evidenced by a 0.01 mil thick electroless copper pattern on each of the three respective film surfaces was obtained.

#### EXAMPLE VI

A. The procedure of Example I-A was repeated except that a 0.1 weight percent aqueous  $\text{AgNO}_3$  solution was prepared. The resultant  $\text{AgNO}_3$  solution was then combined with a colloidal aqueous solution comprising insoluble hydrous oxide particles of zinc, the  $\text{AgNO}_3$  being present in the resultant mixture in a concentration of 0.05 weight percent. The colloidal hydrous zinc oxide solution was prepared in the following manner. One weight percent of zinc chloride [ $\text{ZnCl}_2$ ] was dissolved in 100 ml. of deionized water. A sufficient amount of  $\text{NH}_4\text{OH}$  was then added to the resultant solution to obtain a pH of about 7.0-7.5 to yield a colloidal wetting solution.

A physical development evidenced by a 0.01 mil thick electroless copper pattern on each of the three respective film surfaces was obtained.

B. The procedure of Example VI-A was repeated except that the  $\text{AgNO}_3$  was added to the colloidal solution in a concentration of 0.05 weight percent. The results obtained were the same as in Example VI-A.

#### EXAMPLE VII

A. The procedure of Example I-A was repeated except that a 0.01 weight percent aqueous  $\text{AgNO}_3$  solution was prepared whose pH was adjusted to about 5.2 by the addition of  $\text{HNO}_3$  thereto. The resultant  $\text{AgNO}_3$  solution was then combined with a colloidal aqueous solution comprising insoluble hydrous oxide particles of aluminum. The  $\text{AgNO}_3$  was present in the resultant mixture in a concentration of 0.5 weight percent. The colloidal solution was prepared in the following manner. One weight percent of finely powdered aluminum chloride [ $\text{AlCl}_3$ ] was added to 100 ml. of deionized water. The pH of the resultant solution was raised with  $\text{NaOH}$  to about 5.2. This solution was heated for about 2 hours at about 60-80°C to yield a colorless (milky white) wetting solution.

A physical development evidenced by a 0.01 mil thick electroless copper pattern on each of the three respective film surfaces was obtained.

B. The procedure of Example VII-A was repeated except that the  $\text{AgNO}_3$  was added to the colloidal solution in a concentration of 0.05 weight percent. The results obtained were the same as in Example VII-A.

#### EXAMPLE VIII

10 The procedure of Example I-A was repeated except that a 0.1 weight percent aqueous  $\text{AgNO}_3$  solution was prepared whose pH was adjusted to about 3 by the addition of  $\text{HNO}_3$  thereto. The resultant  $\text{AgNO}_3$  solution was then combined with a colloidal aqueous solution comprising insoluble hydrous oxide particles of indium, the  $\text{AgNO}_3$  being present in the resultant mixture in a concentration of 0.05 weight percent. The colloidal solution was prepared in the following manner. One weight percent of indium trichloride [ $\text{InCl}_3$ ] was dissolved in 100 ml. of deionized water. The pH of this solution was raised to about 3 with  $\text{NaOH}$  yielding a colorless (milky white) wetting solution.

25 A physical development evidenced by a 0.01 mil thick electroless copper pattern on each of the three respective film surfaces was obtained.

#### EXAMPLE IX

A. The procedure of Example I-A was repeated except that a 0.01 weight percent aqueous  $\text{AgNO}_3$  solution was prepared whose pH was adjusted to about 1.0 by the addition of  $\text{HNO}_3$  thereto. The resultant  $\text{AgNO}_3$  solution was then combined with a colloidal aqueous solution comprising insoluble hydrous oxide particles of tin, the  $\text{AgNO}_3$  being present in the resultant mixture in a concentration of 0.05 weight percent. The colloidal solution was prepared in the following manner. One weight percent of stannic chloride [ $\text{SnCl}_4 \cdot 5\text{H}_2\text{O}$ ] was dissolved in 100 ml. of deionized water. The solution was allowed to stand at a temperature of about 60°C for 1 hour until a flocculate formed.

A physical development evidenced by a 0.01 mil thick electroless copper pattern on each of the three respective film surfaces was obtained.

45 B. The procedure of Example IX-A was repeated except that the colloidal solution was prepared in the following manner. One-half weight percent of stannic chloride [ $\text{SnCl}_4 \cdot 5\text{H}_2\text{O}$ ] was dissolved in 100 ml. of deionized water. The resultant solution was allowed to stand for approximately 1 month until the pH thereof was about 0.8-1.8 and a flocculate formed at the bottom thereof. The supernatant portion is a wetting solution. The pH of the  $\text{AgNO}_3$  was adjusted to about 0.8-1.8 by the addition of  $\text{HNO}_3$  thereto and was then combined with the supernatant portion.

55 A physical development evidenced by a 0.01 mil thick electroless copper pattern on each of the three respective film was obtained.

60 C. The procedure of Example IX-A was repeated except that the colloidal wetting solution was prepared in the following manner. The bottom layer containing the flocculate, described in Example IX-B, above, had added thereto sufficient  $\text{HCl}$  to lower the pH to about 0.8-1.8 to yield a colorless (milky white) wetting solution. The results achieved were the same as in Example IX-B, above.

65 D. The procedure of Example IX-B was repeated except that the colloidal wetting solution was prepared in

the following manner. The bottom layer containing the flocculate of the solution of Example IX-B, described above, was heated to 30-90°C for about 30 minutes to yield a colorless (milky white) wetting solution. The results obtained were the same as in Example IX-B, above.

E. The procedure of Example IX-A was repeated except that the colloidal wetting solution was obtained in the following manner. To concentrated HCl was added 2 weight percent of stannic chloride [SnCl<sub>4</sub>.5H<sub>2</sub>O]. The initial pH of this solution was raised to within the range of 0.5-0.8 with NaOH to yield a colloidal wetting solution. The pH of the aqueous AgNO<sub>3</sub> solution was similarly adjusted to 0.5-0.8 by the addition thereto of HNO<sub>3</sub> prior to the combining with the colloidal solution.

A physical development evidenced by a 0.01 mil thick electroless copper pattern on each of the three respective film surfaces was obtained.

F. The procedure of Example IX-A was repeated except that the colloidal wetting solution was prepared in the following manner. To concentrated HBr was added 1-2 weight percent of stannic bromide [SnBr<sub>4</sub>]. The pH of the resultant solution was then raised to within the range of 1.0-1.1 with NaOH. The pH of the aqueous AgNO<sub>3</sub> solution was then lowered to 1.0-1.1 by the addition of HNO<sub>3</sub> thereto prior to combining with the colloidal solution. Upon the combining of the AgNO<sub>3</sub> solution with the colloidal wetting solution a silver bromide, deposit on the colloidal tin hydrous oxide particles was obtained which was photosensitive.

A physical development evidenced by a 0.01 mil thick electroless copper pattern on each of the three respective film surfaces was obtained.

#### EXAMPLE X

A. The procedure of Example I-A was repeated except that a 0.1 weight percent aqueous AgNO<sub>3</sub> solution was prepared whose pH was adjusted to about 1.7-1.9 by the addition of HNO<sub>3</sub> thereto. The resultant AgNO<sub>3</sub> solution was then combined with a colloidal aqueous solution comprising insoluble hydrous oxide particles of iron, the AgNO<sub>3</sub> being present in the resultant mixture in a concentration of 0.05 weight percent. The colloidal solution was prepared in the following manner. One weight percent of ferric chloride [FeCl<sub>3</sub>.6H<sub>2</sub>O] was dissolved in 100 ml. of deionized water. This solution was aided by gradually heating to about 60-80°C and stirring. At a pH of about 1.7-1.9 a tan wetting solution was produced.

A physical development evidenced by a 0.01 mil thick electroless copper pattern on each of the three respective film surfaces was obtained.

B. The procedure of Example X-A was repeated except that the colloidal wetting solution was prepared in the following manner. One-half weight percent of ferric chloride [FeCl<sub>3</sub>.6H<sub>2</sub>O] was dissolved in 100 ml. of deionized water. The final pH of this solution was adjusted to about 1.5-2.0 with HCl. The solution was then heated to 70°C within 20 minutes yielding a coffee-pumpkin color wetting solution.

A physical development evidenced by a 0.01 mil thick electroless copper pattern on each of the three respective film surfaces was obtained.

C. The procedure of Example X-A was repeated except that the colloidal wetting solution was prepared in the following manner. One-half weight percent of ferric

chloride [FeCl<sub>3</sub>.6H<sub>2</sub>O] was dispersed in 100 ml. of deionized water of a final pH of about 1.7-1.9. The solution was allowed to stand in ambient for 1-2 weeks thereby yielding a coffee-pumpkin color wetting solution. Prior to the combining of the AgNO<sub>3</sub> with the resultant wetting solution the aqueous AgNO<sub>3</sub> solution was adjusted to a pH of 1.7-1.9 by the addition of HNO<sub>3</sub> thereto.

A physical development evidenced by a 0.01 mil thick electroless copper pattern on each of the three respective film surfaces was obtained.

D. The procedure of Example X-A was repeated except that the colloidal wetting solution was prepared in the following manner. 100 ml. of deionized water was first heated to 70°C. 1.5-5 weight percent of ferric chloride was added thereto and dissolved therein. The final pH of this wetting solution was 1.5-2.0. The pH of the aqueous AgNO<sub>3</sub> solution was adjusted to 1.5-2.0 by the addition of HNO<sub>3</sub> thereto prior to combining the AgNO<sub>3</sub> with the colloidal solution.

A physical development evidenced by a 0.01 mil thick electroless copper pattern on each of the three respective film surfaces was obtained.

E. The procedure of Example X-A was repeated except that the colloidal wetting solution was prepared in the following manner. 100 ml. of deionized water was heated to 80°C. 1-2 weight percent of ferric chloride was added and the solution was stirred until the ferric chloride dissolved. Upon cooling to 25°C a vermouth colored wetting solution was obtained. The pH of the aqueous AgNO<sub>3</sub> solution was adjusted to 1.3 by the addition of HNO<sub>3</sub> thereto and then combined with the resultant wetting solution.

A physical development evidenced by a 0.01 mil thick electroless copper pattern on each of the three respective film surfaces was obtained.

F. The procedure of Example X-A was repeated except that 0.5 weight percent of sodium bromide (NaBr) was added to the colloidal wetting solution prior to the combination of AgNO<sub>3</sub> therewith. A mixed silver halide salt was obtained, namely, silver bromide and silver chloride, which were deposited on the hydrous oxide colloidal particles to form a photosensitive composition.

G. The procedure of Example X-F was repeated except that 0.5 weight percent of sodium iodide (NaI) was added. A mixed silver chloride, silver iodide deposit was obtained to yield a photosensitive composition.

H. The procedure of Example X-A was repeated except that the colloidal wetting solution was prepared as follows. One weight percent of ferric bromide [FeBr<sub>3</sub>.6H<sub>2</sub>O] was dissolved in 100 ml. of deionized water. The solution was heated to about 60°C for about 16 hours resulting in a colloidal wetting solution having a pH of about 1.8. The aqueous AgNO<sub>3</sub> solution was adjusted to a pH of 1.8 by the addition of HNO<sub>3</sub> thereto and was then combined with the colloidal solution. Silver bromide was deposited or precipitated on the colloidal iron hydrous oxide particles to form a photosensitive composition.

A physical development evidenced by a 0.01 mil thick electroless copper pattern on each of the three respective film surfaces was obtained.

I. The procedure of Example X-H was repeated except that 2.0 weight percent of ferrous iodide [FeI<sub>2</sub>.4H<sub>2</sub>O] was employed. The pH of the resultant colloidal

wetting solution was 2.5. The pH of the aqueous  $\text{AgNO}_3$  solution was adjusted to about 2.5 by the addition of  $\text{HNO}_3$  thereto and was then added to the colloidal wetting solution. Silver iodide was deposited or precipitated on the colloidal iron hydrous oxide particles to form a photosensitive composition.

A physical development evidenced by a 0.01 mil thick electroless copper pattern on each of the three respective film surfaces was obtained.

It is to be understood that the above-described embodiments are simply illustrative of the principles of the invention. Various other modifications and changes may be made by those skilled in the art which will embody the principles of the invention and fall within the spirit and scope thereof.

What is claimed is:

1. A photosensitive silver halide composition comprising a silver halide deposited on colloidal particles of a hydrous oxide of an element selected from the group consisting of Be, Mg, Ti, Zr, V, Cr, Mo, W, Mn, Fe, Co, Ni, Cu, Zn, Cd, Hg, Al, In, Tl, Si, Ge, Sn, Bi, Th, and mixtures thereof.

2. The composition as defined in claim 1 wherein said silver halide comprises silver chloride.

3. A photosensitive silver halide composition comprising silver halide precipitated in the presence of a stable aqueous colloidal wetting solution, formed by a hydrolysis and nucleation reaction, comprising insoluble hydrous oxide particles of an element selected from the group consisting of Be, Mg, Ti, Zr, V, Cr, Mo, W, Mn, Fe, Co, Ni, Cu, Zn, Cd, Hg, Al, In, Tl, Si, Ge, Sn, Bi, Th, and mixtures thereof, said particles having a size within the range of 10A to 10,000A and said hydrolysis reaction including at least (1) dissolution of a salt of said selected element in an aqueous medium and (2) maintenance of the pH of said aqueous medium at a point where no flocculate results.

4. The composition as defined in claim 3 wherein said silver halide comprises silver chloride.

5. A method of forming a wetting photosensitive silver halide composition which comprises combining a suitable silver salt with a stable aqueous colloidal wetting solution, formed by a hydrolysis and nucleation reaction, comprising (a) a halide ion and (b) insoluble hydrous oxide particles of an element selected from the group consisting of Be, Mg, Ti, Zr, V, Cr, Mo, W, Mn, Fe, Co, Ni, Cu, Zn, Cd, Hg, Al, In, Tl, Si, Ge, Sn, Bi,

10 Th, and mixtures thereof, said particles having a size within the range of 10A to 10,000A and said hydrolysis reaction including at least (1) dissolution of a salt of said selected element in an aqueous medium and (2) maintenance of the pH of said aqueous medium at a point where no flocculate results.

6. The method as defined in claim 5 wherein said suitable silver salt comprises  $\text{AgNO}_3$  and said halide ion comprises a chloride ion.

7. A method of rendering a surface photosensitive which comprises:

a. combining a water-soluble silver species with a stable aqueous colloidal wetting solution, formed by a hydrolysis and nucleation reaction, comprising a halide species and insoluble hydrous oxide particles of an element selected from the group consisting of Be, Mg, Ti, Zr, V, Cr, Mo, W, Mn, Fe, Co, Ni, Cu, Zn, Cd, Hg, Al, In, Tl, Si, Ge, Sn, Bi, Th, and mixtures thereof, to precipitate a silver halide and to coat said hydrous oxide particles with said precipitated silver halide; and

b. contacting the surface with said coated particles to deposit a photosensitive film thereof thereon.

8. The method as defined in claim 7 wherein said silver species comprises  $\text{AgNO}_3$  and said halide species comprises chloride ions.

9. In the method of making a photographic image comprising exposing to a light image a photosensitive film comprising silver halide to form a latent image therein, the improvement wherein

the photosensitive film which comprises a silver halide deposited on insoluble colloidal particles of a hydrous oxide of an element selected from the group consisting of Be, Mg, Ti, Zr, V, Cr, Mo, W, Mn, Fe, Co, Ni, Cu, Zn, Cd, Hg, Al, In, Tl, Si, Ge, Sn, Bi, Th, and mixtures thereof.

10. The method as defined in claim 9 wherein said silver halide comprises silver chloride.

11. The method as defined in claim 9 which further comprises treating the exposed film with a suitable developer to develop a visible image therein.

12. The method as defined in claim 9 which further comprises depositing said silver halide deposited colloidal particles on a support medium to form the photosensitive film thereon.

\* \* \* \* \*

# UNITED STATES PATENT OFFICE CERTIFICATE OF CORRECTION

Patent No. 3,854,952 Dated December 17, 1974  
Inventor(s) J. T. Kenney

It is certified that error appears in the above-identified patent and that said Letters Patent are hereby corrected as shown below:

In the specification, Column 1, line 11, "2. 1 Description" should read --2. Description--. Column 2, line 27, "nd Th" should read --and Th--; line 31, "halid" should read --halide--; line 65, "Vol. 11," should read --Vol. II,--. Column 3, line 1, "nd Sons" should read --and Sons--; line 33, "4 to to" should read --to--; line 55, "water 1" should read --water until 1--; line 59, "example" should read --Example--. Column 4, line 13, "0.5-5" should read --0.5-1.5--; line 65, "0.6-8" should read --0.6-0.8--. Column 6, line 32, "CDCl<sub>2</sub>.1/2H<sub>2</sub>O" should read --CdCl<sub>2</sub>.1/2H<sub>2</sub>O--; line 53, "60°C." should read --60°C,--. Column 7, line 24, "1/2 weight" should read --1/2-2 weight--; line 26, "of stand" should read --to stand--.

Column 9, line 14, "ions of" should read --ions to--. Column 11, line 1, "cobalt, The" should read --cobalt, the--; line 33, AgNO<sub>3</sub>" should read --AgNO<sub>3</sub>--; line 37, "0.05" should read --0.5--; line 54, "0.01" should read --0.1--; line 62, "powered" should read --powdered--. Column 12, line 46, "precent" should read --percent--; line 57, "film was" should read --film surfaces was--. Column 14, line 2, "water of" should read --water to--.

In the claims, Column 16, claim 9, line 31, "wherein" should read --wherein:--.

Signed and Sealed this  
twenty-sixth Day of August 1975

[SEAL]

Attest:

RUTH C. MASON  
Attesting Officer

C. MARSHALL DANN  
Commissioner of Patents and Trademarks